# EUROPEAN PATENT SPECIFICATION

(11) **EP 0 586 194 B1**
(45) Date of publication and mention of the grant of the patent: **06.05.1999**
(21) Application number: 93306775.3
(22) Date of filing: 26.08.1993
(51) Int. Cl.: C10M 129/10, C10M 141/00, C10M 141/06, C10M 169/04, C10N 30/10, C10N 40/02, C10N 40/08, C10N 40/25, C10N 40/26

(54) **Antioxidants in high monounsaturated vegetable oils**
Antioxidanten für hoch einfach-ungesättigte pflanzliche Öle
Antioxydants pour huiles végétales hautement mono-insaturées

(30) Priority: 02.09.1992 US 939249
(43) Date of publication of application: 09.03.1994
(73) Proprietor: The Lubrizol Corporation, Wickliffe, Ohio 44092 (US)
(72) Inventor: Carrick, Virginia Anne, Chardon, Ohio 44024 (US); Temel, Cerita, Orange Village, Ohio 44022 (US); Naegely, Paul Carl, Mentor, Ohio 44060 (US)
(74) Representative: Mallalieu, Catherine Louise

(56) References cited:
- EP-A- 0 239 536
- EP-A- 0 456 925
- WO-A-88/05808
- WO-A-93/03123
- GB-A- 2 134 923
- US-A- 5 102 567

## Description

### Field of the Invention

The present invention relates to an anti-oxidant composition for triglyceride oils that contain at least a 70 percent monounsaturated content. Triglyceride oils containing this anti-oxidant composition have utility in hydraulic fluids, two-cycle (two-stroke) internal combustion engines, gear oils, passenger car motor oils and as a food machinery lubricant.

### Background of the Invention

Oxidative stability is an important requirement for all lubricants regardless of their use. Auto-oxidative breakdown is strongly catalyzed by traces of metal ions (especially copper and iron) which become solubilized when the lubricant contacts a metal surface. Organic compounds, particularly those comprising relatively long hydrocarbon segments, and particularly those containing unsaturation, are subject to auto-oxidation when they are contacted with oxygen. This, in turn, results in the deterioration of the base material, often leading to increases in the total acidity, formation of gums, discoloration, loss of physical properties such as tensile strength for resins, or elasticity for elastomers, loss of potency, polymerization rancidity and/or odor.

Various additives are in general added to lubricating oils, hydraulic fluids and lubricating greases in order to improve the performance characteristics of these lubricants. There is in particular, a need for additives which effectively reduce oxidation and ageing of the lubricant, and thus considerably extend the life of the lubricant.

US Patent 5,102,567 (Wolf, April 7, 1992) relates to a lubricating oil provided to lubricate parts such as bearings, gears and slide mechanism particularly in food processing equipment. The food grade lubricating oil provides oxidation, thermal and hydrolytic stability; protects against rusting and corrosion; provides wear protection, prevents foaming; and resists the formation of sludge.

US Patent 4,115,288 (Schmitt, September 19, 1978) is directed to a lubricant composition that is comprised of a major amount of a lubricating oil or grease and as an antiwear agent, a minor amount of a substituted 1,2,3-triazole characterized by the formula: wherein R₁ and R₂ are individually selected from the group consisting of an alkyl group containing from 1 to 18 carbon atoms; an aryl group, such as phenyl; hydrogen; and and where at least one of R₁ and R₂ is other than hydrogen and where n is an integer from 5 to 15.

US Patent 4,746,448 (Kenmochi et al, May 24, 1988) provides a cold rolling oil for steels which comprises (A) 40 to 90 wt % of a monoester of an aliphatic carboxylic acid having 12 to 22 carbon atoms and an aliphatic alcohol having 1 to 12 carbon atoms, (B) 0.5 to 10 wt % of at least one of a dimer acid and a polymerized acid of a higher aliphatic unsaturated acid having 16 to 20 carbon atoms, (C) 2 to 40 wt % of a polyester having a molecular weight of 750 to 7500 and (D) 0.1 to 10 wt % of a polymer compound having nitrogen atoms in a molecule having a molecular weight of 1000 to 100,000.

### Summary of Invention

According to the present invention there is provided an anti-oxidant composition comprising a major amount of
(A) at least one vegetable triglyceride oil of the formula wherein R¹, R² and R³ are aliphatic hydrocarbyl groups having at least 70 percent monounsaturated character and containing from 8 to 24 carbon atoms and a minor anti-oxidant amount of
(B) at least one alkyl phenol of the formula wherein R⁴ is an alkyl group containing from 1 up to 24 carbon atoms and a is 2, and the position para to the OH group is open, and optionally
(D) a metal deactivator selected from
   (1) a benzotriazole of the formula wherein R⁸ is hydrogen or an alkyl group of 1 up to 24 carbon atoms,
   (2) a phosphatide of the formula wherein R⁹ and R¹⁰ are aliphatic hydrocarbyl groups containing from 8 to about 24 carbon atoms, and G is selected from and
   (3) a carbamate of the formula wherein R¹¹ is an alkyl group containing from 1 to 24 carbon atoms, phenyl or alkyl phenyl wherein the alkyl group contains from 1 to 18 carbon atoms, R¹² and R¹³ are hydrogen or an alkyl group containing from 1 to 6 carbon atoms, with the proviso that R¹² and R¹³ are not both hydrogen,
   (4) citric acid and derivatives of citric acid of the formula wherein R¹⁴, R¹⁵ and R¹⁶ are independently hydrocarbon aliphatic hydrocarbyl groups containing from 1 to 12 carbon atoms, with the proviso that at least one of R¹⁴, R¹⁵ and R¹⁶ is an aliphatic hydrocarbyl group,
   (5) a coupled phosphorus-containing amide of the formula wherein X¹, X² and X³, independently is oxygen or sulfur;
      wherein R¹⁷ and R¹⁸, independently is a hydrocarbyl, a hydrocarbyl-based oxy, the hydrocarbyl portions of which contain 6 to 22 carbon atoms, or a hydrocarbyl-based thio, having from 4 to 34 carbon atoms;
      wherein R¹⁹, R²⁰, R²¹ and R²², independently is hydrogen, or an alkyl having from 1 to 22 carbon atoms, or an aromatic, an alkyl-substituted aromatic or an aromatic-substituted alkyl having from 6 to 34 atoms;
      wherein n is zero or 1;
      wherein n' is 2 or 3
      wherein R²³ is hydrogen; and when n' is 2, R²⁴ is selected from -R- and -R'-
      wherein R is an alkyl moiety, in the form of alkylene or alkylidene containing from 1 to 12 carbon atoms and R' is an alkyl moiety, alkylene, alkylidene or carboxyl containing 1 to 60 carbon atoms and when n' is 3, R²⁴ is or
   (6) a methylacrylate derivative formed by the reaction of equal molar amounts of a phosphorus acid of the formula with methylacrylate wherein X¹ and X² are as defined above in (D)(5) and R²⁵ and R²⁶ are each independently a hydrocarbyl, a hydrocarbyl-based thio or preferably a hydrocarbyl-based oxy group wherein the hydrocarbyl portion contains from 1 to 30 carbon atoms and remaining acidity is neutralized with 1 mole propylene oxide for each 20-25 moles of phosphorus acid.

In a preferred embodiment, the invention comprises an anti-oxidant composition comprising a major amount of:
(A) The triglyceride oil as described above with a minor anti-oxidant amount of
(B) at least one alkyl phenol as described above,
(C) at least one aromatic amine of the formula wherein R⁵ is and R⁶ and R⁷ are independently an alkyl group containing from 4 up to 18 carbon atoms and optionally
(D) The metal deactivator as described above.

Various preferred features and embodiments of the present invention will now be described by way of non-limiting example.

### (A) The Triglyceride Oil

In practicing this invention a triglyceride oil is employed which is a vegetable oil of the formula Within the triglyceride formula are aliphatic hydrocarbyl groups having at least 70 percent monounsaturated character and containing from 8 to 24 carbon atoms. The term "hydrocarbyl group" as used herein denotes a radical having a carbon atom directly attached to the remainder of the molecule. The aliphatic hydrocarbyl groups include the following:
(1) Aliphatic hydrocarbon groups; that is, alkyl groups such as heptyl, nonyl, undecyl, tridecyl, heptadecyl; alkenyl groups containing a single double bond such as heptenyl, nonenyl, undecenyl, tridecenyl, heptadecenyl, heneicosenyl; alkenyl groups containing 2 or 3 double bonds such as 8,11-heptadecadienyl and 8,11,14-heptadecatrienyl. All isomers of these are included, but straight chain groups are preferred.
(2) Substituted aliphatic hydrocarbon groups; that is groups containing non-hydrocarbon substituents which, in the context of this invention, do not alter the predominantly hydrocarbon character of the group. Those skilled in the art will be aware of suitable substituents; examples are hydroxy, carbalkoxy, (especially lower carbalkoxy) and alkoxy (especially lower alkoxy), the term, "lower" denoting groups containing not more than 7 carbon atoms.
(3) Hetero groups; that is, groups which, while having predominantly aliphatic hydrocarbon character within the context of this invention, contain atoms other than carbon present in a chain or ring otherwise composed of aliphatic carbon atoms. Suitable hetero atoms will be apparent to those skilled in the art and include, for example, oxygen and sulfur.

The fatty acid moieties are such that the triglyceride has a monounsaturated character of at least 70 percent and preferably at least 80 percent. For example, a triglyceride comprised exclusively of an oleic acid moiety has an oleic acid content of 100% and consequently a monounsaturated content of 100%. Where the triglyceride is made up of acid moieties that are 70% oleic acid, 10% stearic acid, 5% palmitic acid, 7% linoleic and 8% hexadecanoic acid, the monounsaturated content is 78%. It is also preferred that the monounsaturated character be derived from an oleyl radical, i.e., is the residue of oleic acid. The preferred triglyceride oils are high oleic (at least 70percent) acid triglyceride oils. Typical high oleic vegetable oils employed within the instant invention are high oleic safflower oil, high oleic corn oil, high oleic rapeseed oil, high oleic sunflower oil, high oleic soybean oil, high oleic cottonseed oil and high oleic palm olein. A preferred high oleic vegetable oil is high oleic sunflower oil obtained from Helianthus SP available from SVO Enterprises Eastlake, Ohio as Sunyl^{R} high oleic sunflower oil.

### (B) The Alkyl Phenol

Component (B) is at least one alkyl phenol of the formula wherein R⁴ is an alkyl group containing from 1 up to 24 carbon atoms and a is 2. Preferably R⁴ contains from 4 to 18 carbon atoms and most preferably from 4 to 12 carbon atoms. R⁴ may be either straight chained or branched chained and branched chained is preferred. The position para to the OH group is open.

The (B) component is an alkyl phenol, however, mixtures of alkyl phenols may be employed. Preferably the phenol is a butyl substituted phenol containing 2 t-butyl groups. The t-butyl groups occupy the 2,6-position, that is, the phenol is sterically hindered:

### (C) The Aromatic Amine

Component (C) is at least one aromatic amine of the formula wherein R⁵ is and R⁶ and R⁷ are independently an alkyl group containing from 4 up to 18 carbon atoms.

In a particularly advantageous embodiment, component (C) comprises an alkylated diphenylamine such as nonylateddiphenylamine of the formula

### (D) The Optional Metal Deactivator

An optional metal deactivator may be employed wherein the metal deactivator is selected:
(1) a benzotriazole,
(2) a phosphatide,
(3) a carbamate,
(4) citric acid or its derivatives, or
(5) a coupled phosphorus-containing amide.

### (D) (1) The Benzotriazole

A useful metal deactivator is benzotriazole compound of the formula wherein R⁸ is hydrogen a straight or branched-chain alkyl group containing from 1 up to 24 carbon atoms, preferably 1 to 12 carbon atoms and most preferably 1 carbon atom. When R is 1 carbon atom the benzotriazole compound is tolyltriazole of the formula Tolyltriazole is available under the trade name Cobratec TT-100 from Sherwin-Williams Chemical.

### (D) (2) The Phosphatide

Another metal deactivator are the phosphatides of the formula wherein R⁹ and R¹⁰ are aliphatic hydrocarbyl groups containing from 8 to 24 carbon atoms and G is selected from -CH₂CH₂${\text{N}}^{+}$H₃, -CH₂CH₂${\text{N}}^{+}$(CH₃)₃ and Preferably G is -CH₂CH₂${\text{N}}^{+}$(CH₃)₃ such that the phosphatide is lecithin. Particularly effective phosphatides are soybean lecithin, corn lecithin, peanut lecithin, sunflower lecithin, safflower lecithin and rapeseed lecithin.

### (D) (3) The Carbamate

A third useful metal deactivator are the carbamates of the formula wherein R¹¹ is an alkyl group containing from 1 to 24 carbon atoms, phenyl or alkyl phenyl wherein the alkyl group contains from 1 to 18 carbon atoms. Preferably R¹¹ is an alkyl group containing from 1 to 6 carbon atoms. The groups R¹² and R¹³ are hydrogen or an alkyl group containing from 1 to 6 carbon atoms, with the proviso that R¹² and R¹³ are not both hydrogen.

### (D)(4) The Citric Acid and its Derivatives

A fourth useful metal deactivator is citric acid or derivatives of citric acid of the formula wherein R¹⁴, R¹⁵ and R¹⁶ are independently hydrogen or aliphatic hydrocarbyl groups containing from 1 to 12 carbon atoms, with the proviso that at least one of R¹⁴, R¹⁵ and R¹⁶ is an aliphatic hydrocarbyl group and preferably contains from 1 to 6 carbon atoms.

### (D) (5) The Coupled Phosphorus-Containing Amide

The fifth useful metal deactivator is a coupled phosphorus-containing amide that is a statisticalmixture of compounds having the following formula

Considering X¹ and X², it independently is oxygen or sulfur and preferably is sulfur whereas X³ is oxygen or sulfur and preferably oxygen. R¹⁷ and R¹⁸ each independently is a hydrocarbyl, a hydrocarbyl-based thio or preferably a hydrocarbyl-based oxy group wherein the hydrocarbyl portion contains 6 to 22 carbon atoms. The hydrocarbyl portion of R¹⁷ and R¹⁸ generally contains from 1 to 34 carbon atoms. When R¹³ is hydrogen and R²⁴ is methylene, R¹⁷ and R¹⁸ will contain 6 to 12 carbon atoms in order to provide for sufficient oil solubility. The hydrocarbyl portion of R¹⁷ and R¹⁸ independently can be alkyl or aromatic. Although the hydrocarbyl portion of both R¹⁷ and R¹⁸ can be the same type of hydrocarbyl group, that is both alkyl or both aromatic, often one such group can be alkyl and the remaining group can be aromatic. Different coupled phosphorus-containing amide compounds which are made by reacting a mixture of two or more different reactants each containing an alkyl hydrocarbyl group as well as an aromatic hydrocarbyl (R¹⁷ and R¹⁸) group therein. The same or different compounds are coupled via different coupling groups R²⁴ to form a statistical mixture of coupled compounds or are reacted with different compounds to provide different functional groups R²⁴ thereon.

The hydrocarbyl group of R¹⁷ and R¹⁸ is preferably an alkyl containing from 6 to 22 (more preferably 8-12) carbon atoms. Examples of such groups include hexyl, heptyl, octyl, nonyl, decyl, dodecyl, tetradecyl, octadecyl, behenyl, and the like, including all isomers thereof. Should the R¹⁷ or R¹⁸ hydrocarbyl be an aromatic, it can be phenyl or naphthyl. Often times it will have an alkyl substituent thereon. Thus, the alkyl-substituted aromatic can have an alkyl substituent containing from zero, that is phenyl, to 28 carbon atoms, and preferably from 7 to 12 carbon atoms. Whenever a blend of the compounds of coupled phosphorus-containing amide is utilized containing significant or effective amounts of alkyl type R¹⁷ or R¹⁸ substituents, the aromatic substituent can contain preferably from 6 to 12 carbon atoms in the alkyl group thereof, that is, the alkyl-substituted aromatic. This is because although the solubility of phenyl or low alkyl-substituted aromatics may be somewhat low, the overall solubility in a lubricant composition is generally increased to a desirable level through the utilization of the R¹⁷ and R¹⁸ hydrocarbyl portions which are alkyl and/or through the use of R²³ and/or R²⁴ groups which have a large number of carbon atoms therein. The use of lower alkyls, e.g., less than 6 carbon atoms at R¹⁷ and R¹⁸ above with a methylene at R²⁴ is undesirable with respect to oil solubility.

Considering now the alkyl-substituted aromatic group, the aromatic preferably is phenyl while the alkyl can be the same as set forth hereinabove. Specific examples of such alkyl groups on the aromatic nucleus include methyl, ethyl, propyl, butyl, pentyl, heptyl, octyl, decyl, behenyl, and the like including isomers thereof.

Accordingly, specific examples of mixed hydrocarbyl (R¹⁷ and R¹⁸) portions of substituents include tolyl and octyl, tolyl and hexyl, isobutylphenyl and amyl, phenyl and isooctyl, and the like. Mixed hydrocarbyl (R¹⁷ and R¹⁸) substituents are also assured when cresylic acids are utilized to form the phosphorus portion of the coupled phosphorus-containing amide compound. The sources, type and variety of cresylic acids are known to those skilled in the art. The number of different molecular entities in the mixture is further increased by the different coupling groups, R²⁴ as defined above for coupled phosphorus-containing amide when n' is 2 or 3.

When X¹ and X² is sulfur and especially when X² is sulfur, the alkyl hydrocarbyl substituent (R¹⁷ or R¹⁸) contains 6 or more carbon atoms. However, when X¹ or X² is oxygen and especially when X² is oxygen, the alkyl hydrocarbyl substituent (R¹⁷ or R¹⁸) is 6 to 12 carbon atoms.

Considering R¹⁹, R²⁰, R²¹ and R²², each independently can be hydrogen or a saturated hydrocarbyl having up to 22 carbon atoms. The saturated hydrocarbyl group can be an alkyl having from 1 to 22 carbon atoms, a cycloalkyl having from 4 to 22 carbon atoms, or an aromatic, an aromatic-substituted alkyl or an alkyl-substituted aromatic having from 6 to 34 carbon atoms. Preferably, R¹⁹, R²⁰, R²¹ and R²² is hydrogen or methyl with hydrogen being highly preferred. Examples of specific R¹⁹, R²⁰, R²¹ and R²² alkyl groups include methyl, ethyl, propyl, butyl, pentyl, hexyl, heptyl, octyl, nonyl, decyl, dodecyl, tetradecyl, etc., as well as isomers thereof whereas examples of specific aromatic groups include phenyl, tolyl, naphthyl, heptylphenyl, nonylphenyl, dodecylphenyl, wax-substituted phenyl, and the like. With regard to the R²¹-C-R²² group, n can be zero or 1. Preferably n is 1.

Considering now the amide portion of the molecule, R²³ is hydrogen or an alkyl having from 1 to 22 carbon atoms with hydrogen being highly preferred. Examples os specific alkyl groups include methyl, ethyl, propyl, butyl, and so forth including the various isomers thereof.

A particularly preferred embodiment of (D) (5) includes a statistical mixture (i.e., compounds each with different substituent groups providing a variety of different compounds) of different phosphorus containing amide compounds bonded to or couple by different R²⁴ groups with the proviso that in general coupled phosphorus-containing amide the mixture includes some compounds where n' is 2, R²⁴ is Any such statistical mixture is likely to include some coupled amide compounds of coupled phosphorus-containing amide wherein R²⁴ is methylene. When R²⁴ is methylene, R¹⁷ and R¹⁸ generally must contain more than 6 carbon atoms in order to maintain good oil solubility. When n' is 2, R²⁴ is selected from -R- and -R'-
and when n' is 3, R²⁴ is wherein R is independently hydrogen or an alkyl moiety, alkylene or alkylidene of 1 to 12 carbon atoms and R' is hydrogen or an alkyl or carboxy alkyl moiety, alkylene or alkylidene of containing 1 to 60 carbon atoms, R is preferably methylene and R' is preferably an alkyl moiety of 1 to 28 carbons. When R and R' are linking groups, they may be alkylene and/or alkylidene, i.e., the linkage may be vicinal and/or geminal.

The following illustrate the preparation of the coupled phosphorus-containing compounds. All parts and percentages are by weight unless otherwise indicated.

### Example (D) (5)-1

To a mixture of 1775 parts (4.26 equivalents) of O,O-di-isooctyl phosphorodithioic acid and 980 parts of toluene under a nitrogen atmosphere are added 302 parts (4.26 equivalents) of acrylamide. The reaction mixture exotherms to about 56°C and 77 parts (2.33 equivalents) of paraformaldehyde and 215 parts (0.11 equivalent) of p-toluenesulfonic acid hydrate are added. Heating is continued at reflux (92-127°C) while removing 48 parts of water. Upon cooling the mixture to 100°C, 9.2 parts (0.11 equivalent) of sodium bicarbonate is added and cooling continued to about 30°C. A vacuum is applied (15 mm. Hg) and toluene solvent removed while raising the temperature to 110°C. The residue is filtered through a filter aid and the filtrate is the desired product. The product contains 6.86% P (6.74% theory).

### Example (D)(5)-2

To a mixture of 1494 parts (3.79 equivalents) of O,O-di-isooctyl phosphorodithioic acid and 800 parts of toluene under a nitrogen atmosphere are added 537 parts (3.79 equivalents) of 50% aqueous acrylamide solution over a period of one hour. The reaction mixture exotherms to about 53°C and 64 parts (1.93 equivalents) of paraformaldehyde and 18 parts (0.095 equivalent) of p-toluenesulfonic acid hydrate are added. Heating is continued at reflux (91-126°C) for 4 hours while collecting 305 parts of water. The mixture is cooled to about 90°C and 7.6 parts (0.095 equivalent) of 50% aqueous sodium hydroxide solution are added. Cooling is continued to about 30°C and a vacuum is applied (15 mm. Hg). Toluene solvent is removed while raising the temperature to 110°C. The residue is filtered through a filter aid and the filtrate is the desired product. The product contains 6.90% P (6.75% theory) and 2.92% N (2.97% theory).

### Example (D)(5)-3

To a mixture of 984 parts (1.30 equivalents) of O,O-p-di-dodecylphenyl phosphorodithioic acid and 575 parts of toluene under a nitrogen atmosphere are added 100 parts (0.65 equivalent) of methylenebisacrylamide. The reaction mixture exotherms to about 40°C and is heated at 80-85°C for 2 hours. After cooling the mixture to 30°C, a vacuum (15 mm. Hg) is applied and toluene solvent is removed while raising the temperature to 100°C. The residue is filtered through a filter aid and the filtrate is the desired product. The product contains 4.09% P (4.31% theory).

### Example (D) (5)-4

A reaction vessel is charged with 820 parts of toluene and 930 parts (2.32 equivalents) of a O,O-dialkyl phosphorodithioic acid prepared from a mixture of 20 mole percent isobutyl alcohol and 80 mole percent 2-ethylhexyl alcohol. To this mixture under a nitrogen atmosphere are added 178.6 parts (1.16 equivalents) of methylenebisacrylamide. The mixture exotherms to about 65°C and is heated at about 80-85° for 2 hours. Upon cooling to 50°C, a vacuum (30 mm. Hg) is applied. Toluene solvent is removed while raising the temperature to 115°C. The residue is filtered through a filter aid and the filtrate is the desired product. The product contains 7.30% P (7.28% theory).

### Example (D)(5)-5

To a mixture of 305 parts of toluene and 611 parts (1.82 equivalents) of a O,O-di-alkyl-substituted phosphorodithioic acid prepared from a mixture of 20 mole percent phenol and 80 mole percent i-octyl alcohol, are added 258 parts (1.82 equivalents) of a 50% aqueous acrylamide solution over a 20-minute period under a nitrogen atmosphere. After an initial exotherm to 60°C, 32.1 parts (0.97 equivalent) of paraformaldehyde and 7.3 parts (0.038 equivalent) of p-toluenesulfonic acid hydrate are added. The mixture is heated at reflux (91-127°C) for 2 hours while removing 131 parts of water. The mixture is cooled to 80°C and 3.1 parts (0.038 equivalent) of 50% aqueous sodium hydroxide solution is added. Cooling is continued to 50°C and a vacuum (30 mm. Hg) is applied. Toluene solvent is removed while raising the temperature to 110°C. The residue is filtered through a filter aid and the filtrate is the desired product. The product contains 7.09% P (7.42% theory).

### Example (D) (5)-6

To 1017 parts (3.0 equivalents) of O,O-di-4-methyl-2-pentyl phosphorodithioic acid under nitrogen is added 213 parts (3.0 equivalents) of acrylamide. The reaction exotherms to 65°C and held for one to three hours at 65-75°C. The product is filtered through a filter aid and the filtrate is the desired product. The product contains 7.65% P (7.82% theory), 3.51% N (3.50% theory), and 16.05% S (16.06% theory).

### Example (D) (5)-7

To 614 parts (1.5 equivalents) of O,O-di-iso-octyl phosphorodithioic acid under nitrogen is added 213 parts (1.5 equivalents) of a 50% aqueous acrylamide solution. The reaction exotherms to 65°C and held for two hours at 70°C. A vacuum is applied (20 mm. Hg) while raising temperature to 90°C. The residue is filtered through a filter aid and the filtrate is the desired product. The product contains 6.67% P (6.60% theory), 2.94% N (2.97% theory), and 14.50% S (13.60% theory).

### Example (D) (5)-8

To 1340 parts (3.41 equivalents) of O,O-di-isooctyl phosphorodithioc acid under nitrogen is added 242 parts (3.41 equivalents) of acrylamide. The reaction exotherms to 60°C and is held at 65-70°C for one hour. To this mixture are added 400 parts of toluene, 14 parts of potassium carbonate, and 307 parts (3.58 equivalents) of 35% aqueous formaldehyde. The mixture is heated under a nitrogen atmosphere at 35-40°C for 16 hours. To this mixture is added 18.2 parts of glacial acetic acid.

### Example (D) (5)-9

From the product of Example (D)(5)-8, water is removed using a Dean Stark trap at reflux for 6 hours. After 234 parts of water is collected (temperature is 120°C), the mixture is cooled to 30°C. A vacuum is applied (30 mm. Hg) while raising temperature to 115°C. The mixture is filtered through a filter aid and the filtrate is the desired product. The product contains 6.71% phosphorus.

### (D)(6) The Methylacrylate Derivative

The last remaining metal deactivator is a methylacrylate derivative formed by the reaction of equal molar amounts of a phosphorus acid of the formula with methylacrylate wherein X¹ and X² are as defined above in (D) (5) and R²⁵ and R²⁶ are each independently a hydrocarbyl, a hydrocarbyl-based thio or preferably a hydrocarbyl-based oxy group wherein the hydrocarbyl portion contains from 1 to 30 carbon atoms. Preferably R²⁵ and R²⁶ are hydrocarbyl-based oxy groups wherein the hydrocarbyl group contains from 1 to 12 carbon atoms and X¹ and X² are sulfur. Since the reaction does not go to completion, the remaining acidity is neutralized with propylene oxide.

In preparing (D)(6), methylacrylate is added to the phosphorus acid and at the end of this addition, propylene oxide is added. One mole of propylene oxide is employed for every 20-25 moles of phosphorus acid.

The following illustrates the preparation of the methylacrylate derivative. All parts and percentages are by weight unless otherwise indicated.

### Example (D) (6)-1

To 2652 parts (9.04 equivalents) of a O,O-di-alkylphosphorodithioic acid prepared from a mixture of 65 mole percent iso-butyl alcohol and 35 mole percent iso-amyl alcohol is added 776 parts (9.04 equivalents) of methyl acrylate. The methyl acrylate addition is done dropwise and the temperature increases from 60° to 93°C. The contents are held at this temperature for 6 hours and then cooled to 35°C at which 23 parts (0.04 equivalents) propylene oxide is added dropwise. The contents are filtered to give a product having a % phosphorus of 7.54 (8.12% theory).

### RBOT Test

The rotary bomb oxidation test (RBOT) is a relatively short term test method for the oxidation stability of oils.

The RBOT test is a rapid means of estimating the oxidation stability of lubricating oils. In the test, the oil sample, water and a copper catalyst coil are placed in a covered glass container, and placed in a bomb equipped with a pressure gauge. The bomb is charged with oxygen to a pressure of 90 psi (620 Kpa) and placed in a constant temperature oil bath maintained at 150°C and rotated at 100 rpm. The pressure in the bomb is monitored continuously. At first the pressure increases sharply, typically to about 190-200 psi, because of the increase in temperature. The pressure remains relatively stable, until the oil breaks down. The bomb "life" of the sample is the time in minutes from the start of the test to a 25 psi drop from the established plateau pressure. Usually the test uses a 3m length of 14 Awg of copper wire which has been cleaned. The longer the "life", the more stable the oil formulation (i.e., the more effective the anti-oxidant).

The composition of the present invention comprising components (A) and (B) and optionally (D) or (A), (B) and (C) and optionally (D) have utility in hydraulic fluids, two-cycle (two-stroke) internal combustion engines, gear oils, passenger car motor oils and as a food machinery lubricant. The composition of this invention comprises a major amount of (A) and a minor amount (B) and optionally (D) or a major amount of (A) and a minor amount of (B) and (C) and optionally (D). By a major amount is meant more than 50%. Thus 51%, 75% and 99% are major amounts. A minor amount is less than 50%. Examples of minor amounts are 1%, 25% and 49%. The following states the ranges of components (A), (B), (C) and (D) in parts by weight.

| Component | Generally | Preferred | Most Preferred |
|---|---|---|---|
| (A) | 75 - 99 | 85 - 99 | 95 - 99 |
| (B) | 0.1 - 10 | 0.3 - 8 | 0.5 - 5 |
| (C) | 0.1 - 10 | 0.3 - 8 | 0.5 - 5 |
| (D) | 0 - 2 | 0 - 0.5 | 0 - 0.25 |

It is understood that other components besides (A), (B), (C) and (D) may be present within this composition.

The components of this invention are blended together according to the above ranges to effect solutions. The below Table I outlines examples so as to provide those of ordinary skill in the art with a complete disclosure and description on how to make the composition of this invention and it is not intended to limit the scope of what the inventors regard as their invention. All parts are by weight. Where the triglyceride oil, component (A), is identified with a number such as Sunyl^{R} 80 High Oleic Sunflower oil, it means that the oleic acid residue of the triglyceride is 80 percent. In some instances, more than one triglyceride oil is utilized. For example, 80 parts of Sunyl^{R} 90 is blended with normal sunflower oil that contains 20% oleic acid residue to give a sunflower oil blend containing 76% oleic acid residue.

## Claims

1. An anti-oxidant composition for triglyceride oils comprising a major amount of
(A) at least one vegetable triglyceride oil of the formula wherein R¹, R² and R³ are aliphatic hydrocarbyl groups having at least 70 percent monounsaturated character and containing from about 8 to about 24 carbon atoms and a minor anti-oxidant amount of
(B) at least one alkyl phenol of the formula wherein R⁴ is an alkyl group containing from 1 up to 24 carbon atoms, a is 2 and the position para to the OH group is open, and optionally
(D) a metal deactivator selected from
(1) a benzotriazole of the formula wherein R⁸ is hydrogen or an alkyl group of 1 up to 24 carbon atoms,
(2) a phosphatide of the formula wherein R⁹ and R¹⁰ are aliphatic hydrocarbyl groups containing from 8 to 24 carbon atoms, and G is selected from ${\text{-CH}}_{\text{2}} {\text{CH}}_{\text{2}} \text{N} {{\text{H}}^{+}}_{\text{3}} {\text{,-CH}}_{\text{2}} {\text{CH}}_{\text{2}} \text{N(C} {{\text{H}}^{+}}_{\text{3}} {\text{)}}_{\text{3}}$and
(3) a carbamate of the formula wherein R¹¹ is an alkyl group containing from 1 to 24 carbon atoms, phenyl or alkyl phenyl wherein the alkyl group contains from 1 to 18 carbon atoms, R¹² and R¹³ are hydrogen or an alkyl group containing from 1 to 6 carbon atoms, with the proviso and that R¹² and R¹³ are not both hydrogen,
(4) citric acid and derivatives of citric acid of the formula wherein R¹⁴, R¹⁵ and R¹⁶ are independently hydrocarbon or aliphatic hydrocarbyl groups containing form 1 to 12 carbon atoms, with the proviso that at least one of R¹⁴, R¹⁵ and R¹⁶ is an aliphatic hydrocarbyl group,
(5) a coupled phosphorus-containing amide of the fonnula wherein X¹, X² and X³, independently is oxygen or sulfur;
wherein R¹⁷ and R¹⁸, independently is a hydrocarbyl, a hydrocarbyl-based oxy, the hydrocarbyl portions of which contain 6 to 22 carbon atoms, or a hydrocarbyl-based thio, having from 4 to 34 carbon atoms;
wherein R¹⁹, R²⁰, R²¹ and R²², independently is hydrogen, or an alkyl having from 1 to 22 carbon atoms, or an aromatic, an alkyl-substituted aromatic or an aromatic-substituted alkyl having from 6 to 34 atoms;
wherein n is zero or 1;
wherein n' is is or 3
wherein R²³ is hydrogen; and when n' is 2, R²⁴ is selected from -R- and -R'-
wherein R is an alkyl moiety, in the form of alkylene or alkylidene containing form 1 to 12 carbon atoms and R' is an alkyl moiety, alkylene, alkylidene or carboxyl containing 1 to 60 carbon atoms and when n' is 3, R²⁴ is or
(6) a methylacrylate derivative prepared by reacting equal molar amounts of a phosphorus acid of the formula with methylacrylate wherein X¹ and X² are oxygen or sulfur and R²⁵ and R²⁶ are each independently a hydrocarbyl, a hydrocarbyl-based thio or a hydrocarbyl-based oxy group wherein the hydrocarbyl portion contains from 1 to 30 carbon atoms and remaining acidity is neutralized with 1 mole propylene oxide for each 20-25 moles of phosphorus acid.

2. The composition of claim 1 wherein the vegetable oil triglyceride is an ester of at least one straight chain fatty acid and glycerol wherein the fatty acid contains from about 8 to 22 carbon atoms.

3. The composition of claim 1 or claim 2 wherein the monounsaturated fatty acid is oleic acid.

4. The composition of any preceding claim wherein a is 2 and R⁴ contains from 1 up to 8 carbon atoms.

5. The composition of claim 4 wherein the alkyl phenol is of the formula wherein R⁴ is t-butyl.

6. The composition of any preceding claim wherein R⁸ is hydrogen or an alkyl group containing from 1 up to 8 carbon atoms.

7. The composition of claim 6 wherein R⁸ is a methyl group.

8. The composition of any preceding claim wherein R⁶ and R⁷ are nonyl groups.

9. The composition of any preceding claim wherein X¹ and X² are sulfur and R²⁵ and R²⁶ are hydrocarbyl-based oxy groups wherein the hydrocarbyl group contains from 1 to 12 carbon atoms.

10. The composition of any preceding claim containing from 75-99 parts by weight (A), 0.1-10 parts by weight (B) and optionally from 0-2 parts by weight (D).

11. The composition of any one of claims 1 to 9 further comprising
(C) at least one aromatic amine of the formula wherein R⁵ is and R⁶ and R⁷ are alkyl groups containing from 4 up to 18 carbon atoms.

12. The composition of claim 11 containing from 75-99 parts by weight (A), 0.1-10 parts by weight (B), from 0.1-10 parts by weight (C) and optionally from 0-2 parts by weight (D).

13. A process for preparing a composition according to any preceding claim comprising blending together a major amount of (A) the vegetable triglyceride oil and a minor amount of (B) the alkyl phenol and optionally (D) the metal deactivator and (C) the aromatic amine.

## Patentansprüche

1. Antioxidationsmittelzusammensetzung für Triglyceridöle, umfassend eine Hauptmenge von
(A) mindestens einem pflanzlichen Triglyceridöl der allgemeinen Formel in der R¹, R² und R³ aliphatische Hydrocarbylreste mit mindestens 70% einfach ungesättigtem Charakter sind und 8 bis 24 Kohlenstoffatome enthalten, und eine geringere Antioxidationsmittelmenge von
(B) mindestens einem Alkylphenol der allgemeinen Formel in der R⁴ ein Alkylrest, enthaltend 1 bis 24 Kohlenstoffatome ist, a gleich 2 ist und die Position para zur OH-Gruppe frei ist, und wahlweise
(D) einem Metalldeaktivator, ausgewählt aus
(1) einem Benzotriazol der allgemeinen Formel in der R⁸ ein Wasserstoffatom oder ein Alkylrest mit 1 bis 24 Kohlenstoffatomen ist,
(2) einem Phosphatid der allgemeinen Formel in der R⁹ und R¹⁰ aliphatische Hydrocarbylreste enthaltend 8 bis 24 Kohlenstoffatome sind, und G ausgewählt ist aus ${\text{-CH}}_{\text{2}} {\text{CH}}_{\text{2}} \text{N} {{\text{H}}^{+}}_{\text{3}} {\text{,-CH}}_{\text{2}} {\text{CH}}_{\text{2}} \text{N(C} {{\text{H}}^{+}}_{\text{3}} {\text{)}}_{\text{3}}$und
(3) einem Carbamat der allgemeinen Formel in der R¹¹ ein Alkylrest enthaltend 1 bis 24 Kohlenstoffatome ist, Phenyl oder Alkylphenyl ist, wobei der Alkylrest 1 bis 18 Kohlenstoffatome enthält, R¹² und R¹³ Wasserstoffatome oder ein Alkylrest enthaltend 1 bis 6 Kohlenstoffatome sind, mit der Maßgabe, daß R¹² und R¹³ nicht beide Wasserstoffatome sind,
(4) Zitronensäure und Derivate von Zitronensäure der allgemeinen Formel in der R¹⁴, R¹⁵ und R¹⁶ unabhängig Kohlenwasserstoff- oder aliphatische Hydrocarbylreste enthaltend 1 bis 12 Kohlenstoffatome sind, mit der Maßgabe, daß mindestens einer der Reste R¹⁴, R¹⁵ und R¹⁶ ein aliphatischer Hydrocarbylrest ist,
(5) einem gekoppelten Phosphor-enthaltenden Amid der allgemeinen Formel
in der X¹, X² und X³ unabhängig ein Sauerstoffatom oder Schwefelatom ist;
in der R¹⁷ und R¹⁸ unabhängig ein Hydrocarbylrest, ein Oxyrest auf Hydrocarbylbasis ist, wobei die Hydrocarbylanteile 6 bis 22 Kohlenstoffatome enthalten, oder ein Thiorest auf Hydrocarbylbasis mit 4 bis 34 Kohlenstoffatomen ist;
in der R¹⁹, R²⁰, R²¹ und R²² unabhängig ein Wasserstoffatom oder ein Alkylrest mit 1 bis 22 Kohlenstoffatomen ist, oder ein aromatischer, ein Alkyl-substituierter aromatischer oder ein aromatisch-substituierter Alkylrest mit 6 bis 34 Atomen ist;
in der n gleich 0 oder 1 ist;
in der n' gleich 2 oder 3 ist;
in der R²² ein Wasserstoffatom ist; und falls n' gleich 2 ist, wird R²⁴ ausgewählt aus -R- und -R'-
wobei R ein Alkylrest in Form eines Alkylens oder Alkylidens enthaltend 1 bis 12 Kohlenstoffatome ist und R' ein Alkyl-, Alkylen-, Alkyliden- oder Carboxylrest enthaltend 1 bis 60 Kohlenstoffatome ist und falls n' gleich 3 ist, ist R²⁴ oder
(6) einem Methylacrylatderivat, hergestellt durch Umsetzung von äquimolaren Mengen einer Phosphorsäure der allgemeinen Formel mit Methylacrylat, wobei X¹ und X² Sauerstoff- oder Schwefelatome sind und R²⁵ und R²⁶ jeweils unabhängig ein Hydrocarbylrest, ein Thio- oder Oxyrest auf Hydrocarbylbasis ist, wobei der Hydrocarbylteil 1 bis 30 Kohlenstoffatome enthält und die restliche Azidität mit einem Mol Propylenoxid pro 20 bis 25 Mol Phosphorsäure neutralisiert wird.

2. Zusammensetzung gemäß Anspruch 1, wobei das pflanzliche Triglyceridöl ein Ester von mindestens einer geradkettigen Fettsäure und Glycerin ist, wobei die Fettsäure etwa 8 bis 22 Kohlenstoffatome enthält.

3. Zusammensetzung gemäß Anspruch 1 oder Anspruch 2, wobei die einfach ungesättigte Fettsäure Ölsäure ist.

4. Zusammensetzung gemäß einem der vorstehenden Ansprüche, wobei a gleich 2 ist und R⁴ 1 bis 8 Kohlenstoffatome enthält.

5. Zusammensetzung gemäß Anspruch 4, wobei das Alkylphenol die allgemeine Formel besitzt, in der R⁴ t-Butyl ist.

6. Zusammensetzung gemäß einem der vorstehenden Ansprüche, wobei R⁸ ein Wasserstoffatom oder ein Alkylrest enthaltend 1 bis 8 Kohlenstoffatome ist.

7. Zusammensetzung gemäß Anspruch 6, wobei R⁸ ein Methylrest ist.

8. Zusammensetzung gemäß einem der vorstehenden Ansprüche, wobei R⁶ und R⁷ Nonylreste sind.

9. Zusammensetzung gemäß einem der vorstehenden Ansprüche, wobei X¹ und X² Schwefelatome sind und R²⁵ und R²⁶ Oxyreste auf Hydrocarbylbasis sind, wobei der Hydrocarbylrest 1 bis 12 Kohlenstoffatome enthält.

10. Zusammensetzung gemäß einem der vorstehenden Ansprüche, enthaltend 75-99 Gewichtsteile (A), 0,1-10 Gewichtsteile (B) und wahlweise 0-2 Gewichtsteile (D).

11. Zusammensetzung gemäß einem der Ansprüche 1 bis 9, weiter umfassend
(C) mindestens ein aromatisches Amin der allgemeinen Formel in der R⁵ ist und R⁶ und R⁷ Alkylreste enthaltend 4 bis 18 Kohlenstoffatome sind.

12. Zusammensetzung gemäß Anspruch 11, enthaltend 75-99 Gewichtsteile (A), 0,1-10 Gewichtsteile (B), 0,1-10 Gewichtsteile (C) und wahlweise 0-2 Gewichtsteile (D).

13. Verfahren zur Herstellung einer Zusammensetzung gemäß einem der vorstehenden Ansprüche, umfassend Zusammenmischen einer Hauptmenge von (A) des pflanzlichen Triglyceridöls und einer geringeren Menge von (B) des Alkylphenols und wahlweise (D) des Metalldeaktivators und (C) des aromatischen Amins.

## Revendications

1. Une composition d'anti-oxydant pour huiles de triglycérides comprenant une quantité majeure de
(A) au moins une huile végétale de triglycéride de la formule où R¹, R² et R³ sont des groupes hydrocarbyle aliphatique ayant au moins 70 pour cent de caractère mono-insaturé et contenant de 8 à 24 atomes de carbone et une quantité anti-oxydante mineure de
(B) au moins un alcoyl phénol de la formule où R⁴ est un groupe alcoyle contenant de 1 à 34 atomes de carbone, a est 2 et la position para par rapport au groupe OH est libre, et facultativement
(D) un désactivateur de métaux choisi parmi
(1) un benzotriazole de la formule où R⁸ est de l'hydrogène ou un groupe alcoyle de 1 à 24 atomes de carbone,
(2) un phosphatide de la formule où R⁹ et R¹⁰ sont des groupes hydrocarbyle aliphatique contenant de 8 à 24 atome de carbone et G est choisi parmi ${\text{-CH}}_{\text{2}} {\text{CH}}_{\text{2}} \text{N} {{\text{H}}^{+}}_{\text{3}} {\text{,-CH}}_{\text{2}} {\text{CH}}_{\text{2}} \text{N(C} {{\text{H}}^{+}}_{\text{3}} {\text{)}}_{\text{3}}$et
(3) un carbamate de la formule où R¹¹ est un groupe alcoyle contenant de 1 à 24 atomes de carbone, phényle ou alcoyl phényle où le groupe alcoyle contient de 1 à 18 atomes de carbone, R¹² et R¹³ sont de l'hydrogène ou des groupes alcoyle contenant de 1 à 6 atomes de carbone, avec le condition que R¹² et R¹³ ne sont pas tous deux de l'hydrogène,
(4) l'acide citrique et des dérivés d'acide citrique de la formule où R¹⁴, R¹⁵ et R¹⁶ sont chacun indépendamment un groupe d'hydrocarbure ou hydrocarbyle aliphatique contenant de 1 à 12 atomes de carbone, avec la condition qu'au moins un de R¹⁴, R¹⁵ et R¹⁶ est un groupe hydrocarbyle aliphatique
(5) un amide phosphoré couplé de la formule où X¹, X² et X³ indépendamment sont chacun de l'oxygène ou du soufre ;
où R¹⁷ et R¹⁸ sont chacun indépendamment un groupe hydrocarbyle ou hydrocarbyl-oxy, dont les portions hydrocarbyle contiennent de 6 à 22 atomes de carbone, ou un groupe hydrocarbyl-thio, ayant de 4 à 34 atomes de carbone ;
où R¹⁹, R²⁰, R²¹ et R²² sont chacun indépendamment un atome d'hydrogène ou un groupe alcoyle ayant de 1 à 22 atomes de carbone ou un groupe aromatique, un groupe aromatique alcoylé ou un groupe alcoyle à substituant aromatique ayant de 6 à 34 atomes de carbone :
où n est zéro ou 1 ;
où n' est 2 ou 3 ;
où R²³ est de l'hydrogène et, quand n' est 2, R²⁴ est choisi parmi -R-; et -R'-
où R est une portion alcoyle, sous la forme d'un groupe alcoylène ou alcoylidène contenant de 1 à 12 atomes de carbone et R'est une portion alcoyle, alcoylène ou alcoylidène ou carboxyle contenant de 1 à 60 atomes de carbone et quand n' est 3, R²⁴ est
(6) un dérivé d'acrylate de méthyle préparé en faisant réagir des quantités molaires égales d'un acide du phosphore de la formule avec l'acrylate de méthyle, où X¹ et X² sont de l'oxygène ou du soufre et R²⁵ et R²⁶ sont chacun indépendamment un groupe hydrocarbyle, un groupe hydrocarbyl-thio ou un groupe hydrocarbyl-oxy dont la portion hydrocarbyle contient de 1 à 10 atomes de carbone et l'acidité restante est neutralisée par 1 mole d'oxyde de propylène pour 20-25 moles d'acide du phosphore.

2. La composition selon la revendication 1, dans laquelle le triglycéride de l'huile végétale est un ester d'au moins un acide gras à chaîne droite et de glycérol, où l'acide gras contient d'environ 8 à 22 atomes de carbone.

3. La composition selon la revendication 1 ou 2, dans laquelle l'acide gras mono-insaturé est l'acide oléique.

4. La composition selon l'une quelconque des revendications précédentes, dans laquelle a est 2 et R⁴ contient de 1 à 8 atomes de carbone.

5. La composition selon la revendication 4, dans laquelle l'alcoyl phénol est de la formule où R⁴ est un groupe t-butyle.

6. La composition selon l'une quelconque des revendications précédentes, dans laquelle R⁸ est de l'hydrogène ou un groupe alcoyle contenant de 1 à 8 atomes de carbone.

7. La composition selon la revendication 6, dans laquelle R⁸ est un groupe méthyle.

8. La composition selon l'une quelconque des revendications précédentes, dans laquelle R⁶ et R⁷ sont des groupes nonyle.

9. La composition selon l'une quelconque des revendications précedentes, dans laquelle X¹ et X² sont du soufre et R²⁵ et R²⁶ sont des groupes hydrocarbyl-oxy dans lesquels le groupe hydrocarbyle contient de 1 à 12 atomes de carbone.

10. La composition selon l'une quelconque des revendications précédentes, contenant de 75 à 99 parties en poids de (A), de 0,1 à 10 parties en poids de (B) et éventuellement de 0 à 2 parties en poids de (D).

11. La composition selon l'une quelconque des revendications 1 à 9, comprenant en outre
(C) au moins une amine aromatique de la formule où R⁵ est et R⁶ et R⁷ sont des groupes alcoyle contenant de 4 à 10 atomes de carbone.

12. La composition selon la revendication 11, contenant de 75 à 99 parties en poids de (A), de 0,1 à 10 parties en poids de (B), de 0,1 à 10 parties en poids de (C) et éventuellement de 0 à 2 parties en poids de (D).

13. Un procédé de préparation d'une composition selon l'une quelconque des revendications précédentes, comprenant le mélange ensemble d'une quantité majeure de (A), l'huile végétale de triglycéride, et d'une quantité mineure de (B), l'alcoyl phénol, et éventuellement de (D), le désactivateur de métaux, et de (C), l'amine aromatique.
